

(No Model.)

I. DE V. WARNER.  
MANUFACTURE OF DRESS STIFFENERS.

No. 403,160.

Patented May 14, 1889.



### Witnesses.

John G. Hinkel, Jr.  
C. S. M. Arthur

Da dev Wamer  
Inventor.  
By Jester & Freeman

Inventor,

Attorneys.

# UNITED STATES PATENT OFFICE.

IRA DE VER WARNER, OF BRIDGEPORT, CONNECTICUT.

## MANUFACTURE OF DRESS-STIFFENERS.

SPECIFICATION forming part of Letters Patent No. 403,160, dated May 14, 1889.

Application filed September 29, 1888. Serial No. 286,759. (No model.)

*To all whom it may concern:*

Be it known that I, IRA DE VER WARNER, a citizen of the United States, residing at Bridgeport, county of Fairfield, State of Connecticut, have invented a new and useful Improvement in the Manufacture of Dress-Stiffeners, of which the following is a full, clear, and exact specification.

Frequent attempts have been made to produce from bundled fibers a stiffening-blade which will serve in every respect as a substitute for whalebone. Success has been attained to the extent of producing stiffening-blades capable of being effectively employed for many purposes for which whalebone, horn strips, &c., have been used, as in dress-stiffeners, panniers, &c.; but before my invention no blade has been produced which can be effectively employed like a whalebone blade for insertion in the pocket of a corset after the corset-body has been made. One reason of the failure to produce the required article has been the difficulty of binding together a series of crooked fibers in such manner that each shall lie substantially straight and parallel to the others and to the straight sides of the finished blade. I have discovered that by using cords or bundles in which the fibers are arranged longitudinally as nearly straight and parallel as practicable in view of their curved and crooked condition and applying a sufficient tension to two or more of such bundles of fibers and then binding them together while under such tension the fibers are all straightened and brought parallel to each other, so that the application of the binding confines each to the other. The tendency of any fibers to spring to one side is counteracted by that of others to bend in the opposite direction, so that however crooked the individual fibers may be a perfectly straight blade is produced.

Different means may be employed for applying the tension to the fibers, as will be obvious to any skilled mechanic; but I will now describe those which in practice have proved very effective, reference being had to the accompanying drawings, in which—

Figure 1 is an elevation in section of a machine for carrying out my improvement. Fig. 2 is a plan of Fig. 1. Fig. 3 is a sectional

view illustrating a press for condensing and tempering the material.

The frame A of the machine may be constructed to support one or a series of similar devices, one being shown, and it has bearings for the journals of a shaft carrying two delivery-reels, B B', and also for a reel, C, the construction being such as to permit the ready removal and replacement of each reel.

To the platform 2 of the frame, in a line between the reels B, B', and C, is secured an overlaying or thread-winding machine, D, constructed in any suitable manner—for instance, as set forth in Letters Patent to J. A. House, No. 259,158—so that two threads are wound in opposite directions upon the double strip passing through the machine D.

Upon each reel B or B' is wound a cord, a, consisting of a bundle of fibers, preferably bound together as set forth in the Letters Patent issued to Warner and Tallman, No. 234,757, and the two cords from the two reels B B' are brought parallel and then bound together by any suitable binding material.

Thus they may be bound by threads as they are carried side by side through the overlaying or binding machine D, from which they pass as one cord to the receiving-reel C. A determined resistance is applied in any suitable manner to the passage of each cord or bundle a of fibers to the reel C, so as to create a tension upon the cords that will straighten out the fibers, bring them parallel to each other, and maintain them thus until tightly bound together by the threads from the overlaying-machine. Thus at the side of each reel B B' is a band-wheel, 3, over which passes a friction or brake strap, 4, secured at one end to an eyebolt, 5, and carrying at the other a weight, 6, capable of being varied. The reel C is driven so as to exert a draft upon the cords sufficient to draw them at the desired speed through the machine D, or the latter may have feed-rolls, as usual. One mode of driving the reel C is shown, and consists of an endless belt, 7, passing from a driving-wheel, 8, round guide-pulleys 9 9, and round a band-wheel, 10, secured to the side of the reel C.

The driving-wheel 8 is secured to a driving-shaft carrying a double pulley, 12, from which bands 13 14 pass to the pulleys of the machine

D, the shaft 15 being driven from any suitable source of power.

In order to prevent the unwinding of the overlaying threads or material binding the fibers together and to also secure a better surface finish, I apply a cement or paste to such overlaying or binding material or to the surface of the bundle that will cause the adhesion of the binding to the bundle of fibers. Thus, 10 as illustrating one mode of applying cement, I use two wells or troughs, each having a pasting-roller, 19, rotating in contact with the traveling cord, and carrying to the surface thereof a thin layer of cement that secures the binding material to the fibers without penetrating to any considerable extent the interstices between the fibers. Tension is thus applied independently to each cord or bundle of fibers, so as to straighten the same, the two bundles 15 are brought side by side and then tightly bound together in one cord by suitable overlaying material, and the latter is then cemented to the faces of the fibers. By thus applying tension to each bundle of fibers separately 20 each is drawn to the extent needed to straighten its fibers, so that when brought against the other bundle the two will be perfectly parallel, and when the binding is applied the fibers will be confined in the straight 25 position to which they were brought, and the compound cord thus produced is perfectly straight, composed of substantially straight parallel fibers, in contradistinction to the bent and twisted cords produced by binding together bundles of fibers without tension, as 30 heretofore. After the compound cord is thus made (two or more bundles of fibers being employed) it is flattened by compression for a determined time between heated dies, the 35 fibers when of "tampico" or "ixtle" being thus also tempered. This may be effected in any suitable press. Thus the cord  $x$  may be cut into suitable lengths, and the latter may be placed between the steam-heated plates 20

21 of a powerful press, F, and held under 45 pressure until the desired effect is produced.

I do not limit myself to the form of drawing or stretching, binding, and pressing machines described, as other forms may be used in carrying out my invention. 50

I do not here claim the corset-stiffener constituting the product of the method of manufacture herein set forth, as the same constitutes the subject of a separate application for Letters Patent, Serial No. 286,760. 55

I claim—

1. The within-described improvement in the art of manufacturing stiffening-blades, the same consisting in arranging fibers longitudinally in bundles and then bringing two 60 or more of said bundles parallel side by side and binding them together under tension, whereby the fibers of said bundles are brought into substantially parallel straight lines and held in this condition, substantially as set 65 forth.

2. The within-described process of forming stiffening-blades, consisting in arranging fibers longitudinally in bundles and arranging two or more of said bundles parallel side 70 by side, binding them together under tension, and subjecting the compound bundle to heat and pressure, substantially as set forth.

3. In the manufacture of stiffening-blades, arranging fibers longitudinally in bundles, 75 bringing two or more of said bundles together parallel side by side, binding them together under tension, coating the same with cement, and flattening under heat and pressure, substantially as set forth. 80

In testimony whereof I have signed my name to this specification in the presence of two subscribing witnesses.

IRA DE VER WARNER.

Witnesses:

F. S. ANDREWS,  
W. P. LANDON.